

# UNITED STATES PATENT OFFICE.

ANTHONY W. O'BLENUS, OF NEW YORK, N. Y.

## STAINING COMPOUND FOR WOOD.

SPECIFICATION forming part of Letters Patent No. 270,833, dated January 16, 1883.

Application filed November 4, 1882. (Specimens.)

*To all whom it may concern:*

Be it known that I, ANTHONY W. O'BLENUS, a citizen of the United States, residing at New York, in the county and State of New York, 5 have invented new and useful Improvements in Staining Compounds for Wood, of which the following is a specification.

This invention relates to a compound prepared of stearic acid, boiled-oil colors, dry coloring-matter, and resin, said ingredients being mixed together, as hereinafter described.

In carrying out my invention I take stearic acid, ten pounds; boiled-oil color, one and one-half pound; dry coloring-matter, one and one-half pound; resin, one-fourth pound. The boiled-oil color which I use is prepared by mixing powdered sienna, ocher, red vermillion or amber with boiled linseed-oil in the usual manner. The dry coloring-matter, which is powdered 15 sienna, ocher, red vermillion or amber, is used in a pulverulent state, and must be of the same 20 nature as the coloring-matter used in preparing the boiled-oil color.

In mixing the ingredients together I proceed as follows: The stearic acid is melted, 25 and then the boiled color is stirred into it, so as to produce a homogeneous mass. When this has been accomplished the mass is permitted to cool, and it is then reduced to a fine 30 powder. This powder is intimately mixed with the dry coloring-matter and with the resin, both the coloring-matter and the resin having been previously reduced to a powder.

When my staining compound is applied to wood—for instance, to a wooden floor—it enters the grain of the wood and produces a fine 35 glossy finish, while at the same time the resin prevents the surface of the floor from becoming slippery.

In preparing my staining compound it is 40 requisite to follow the instructions hereinbefore stated, for I have not been able to obtain a good result by mixing all the ingredients together at once; but I have found that by mixing the boiled-oil color with the stearic acid, 45 then reducing the mixture to a fine powder, and mixing this powder with the remaining ingredients the desired result is reached.

What I claim as new, and desire to secure by Letters Patent, is—

1. A staining compound made of stearic acid, boiled-oil color, dry coloring-matter, and resin, substantially as hereinbefore described.

2. The within-described process for producing a staining compound for wood by mixing 55 stearic acid with boiled-oil color, then reducing the mixture to a fine powder, and mixing this powder with dry coloring-matter and resin about in the proportion hereinbefore stated.

In testimony whereof I have hereunto set my 60 hand and seal in the presence of two subscribing witnesses.

ANTHONY W. O'BLENUS. [L. S.]

Witnesses:

W. HAUFF,

E. F. KASTENHUBER.